

June 7, 1966

P. J. CLOUGH ET AL

3,255,035

TIN OXIDE COATING

Filed Nov. 15, 1961



Fig. 1



Fig. 2

# United States Patent Office

3,255,035

Patented June 7, 1966

1

## 3,255,035 TIN OXIDE COATING

Philip J. Clough, Reading, Paul L. Raymond, Beverly, and Robert W. Steeves, Nahant, Mass., assignors, by mesne assignments, to National Research Corporation, Cambridge, Mass., a corporation of Massachusetts

Filed Nov. 15, 1961, Ser. No. 152,550  
5 Claims. (Cl. 117—62)

The present invention relates to coating and more particularly to a method of coating nonmetallic substrates with tin metal.

In the past considerable effort and attention has been directed to the vacuum vapor deposition of aluminum metal on nonmetallic substrates to produce bright specular metallic coatings for use in products requiring a high quality specular metallic appearance. The use of tin metal for providing such coatings has not been desirable since the tin coatings produced by thermal evaporation in a vacuum chamber were of poor quality. Heretofore tin coatings produced by vacuum deposition methods resulted in coatings which were, for example, milky white, hazy, or brown and non specular in appearance.

Accordingly, it is a principal object of the present invention to provide a method of depositing tin coatings of high specular metallic appearance on nonmetallic substrates by thermal evaporation in a vacuum chamber.

Another object of the present invention is to provide a method of producing coated transparent nonmetallic sheets, ribbons, and threads having a specular metallic appearance and which are highly resistant to dyeing solutions particularly alkaline dye solutions.

Other objects of the invention will in part be obvious and will in part appear hereinafter.

The present invention accordingly comprises the product possessing the features, properties, and the relation of components and the process involving the several steps and the relation and the order of one or more of such steps with respect to each of the others which are exemplified in the following detailed disclosure, and the scope of the application of which will be indicated in the claims.

For a fuller understanding of the nature and objects of the invention, reference should be had to the following detailed description taken in connection with the accompanying drawings wherein:

FIG. 1 is an enlarged, diagrammatic, schematic view of one embodiment of the invention.

FIG. 2 is an enlarged schematic, cross-section of another embodiment of the invention.

The method of depositing bright, specular coatings of tin on a non-metallic flexible substrate by thermal evaporation in a vacuum chamber, in accordance with the present invention, consists in sufficiently evacuating the chamber to provide a residual gas pressure below about 100 microns Hg abs., heating tin metal in a container to a temperature in excess of about 1400° C. to provide an evaporation rate of tin in excess of about 2 grams per minute per square inch of molten tin surface, positioning the substrate in the path of the tin vapors and moving the substrate across the tin vapor path. In this manner the tin vapors condense on the substrate in the form of a highly specular film of superior quality.

Furthermore, in accordance with the present invention, it has been discovered that when the deposition is carried out at a residual chamber pressure in excess of about 100 microns Hg abs. the quality of the tin coating is inferior with respect to brightness and specular appearance. It has further been discovered that when the evaporation rate of the tin metal is less than about 2 grams per minute per square inch of molten tin surface the deposit becomes darkened and non-specular.

2

Thus, maintaining a residual gas pressure in the chamber of below about 100 microns Hg abs. and heating the tin metal to a temperature in excess of about 1400° C. to provide an evaporation rate of tin in excess of about 5 2 grams per minute per square inch of molten tin surface comprise important features of practicing the present invention.

While the tin is initially deposited it is strongly adherent; however, its resistance to abrasion is very slight 10 and the tin coating can be easily smudged or scratched. Accordingly the invention also comprises treatment of the tin coating to improve its resistance to abrasion. The tin film is preferably oxidized immediately to provide at least a surface film of tin oxide.

15 The hardening or oxidizing treatment, in accordance with the present invention, comprises subjecting the tin coating to hot humid or moist air for a period of about 4 minutes or to condensing steam for a period of about 20 seconds. Hot humid air or condensing steam is of particular advantage where the substrate consists of paper and where it is desired to condition the paper by introducing a predetermined amount of moisture. Thus the hardening process of the present invention can serve a dual 25 purpose. Also it has been determined that the hardening process can be accelerated by subjecting the tin coating to dry steam for a period of about 10 seconds.

In a preferred embodiment of the invention for coating flexible transparent plastic sheets, the tin source temperature is such that about 6 grams of tin are evaporated per 30 minute per square inch of molten tin surface in the source. This high evaporation rate gives a shiny, dense, specularly reflecting tin film. The vacuum in the chamber is preferably maintained at a pressure on the order of 10 to 100 microns Hg abs. which provides for economical coating operations, particularly with semicontinuous coaters. The thickness of the tin deposited is preferably between about 35 1 and 5 millionths of an inch. This corresponds approximately to a measured resistivity of between 5 and 1 ohm per square. Coatings much in excess of 5 millionths of an inch do not add to the appearance of the product and are more expensive. Coatings much less than 1 millionth of an inch are, for most purposes, too transparent. The rate of travel of the substrate through the tin vapors or the time of exposure of the substrate can be varied in 40 45 relation to the rate of evaporation in order to achieve the desired coating thickness. The tin coating deposited is then treated as described above to improve its resistance to abrasion.

Where a laminated product is desired, the tin-coated 50 plastic sheet is then laminated to another transparent plastic sheet which can be of the type normally used for making such plastic-metallic threads as fully described in the Prindle and Lacy Patent 2,714,569. This lamination is preferably achieved by use of suitable thermoplastic 55 adhesives which may include dyes or other materials for producing special optical effects.

Referring now to the drawings there are illustrated several preferred embodiments of the invention. In FIGURE 1 the base sheet is indicated at 10 as carrying a thin 60 layer of tin 12. Adjacent to the tin layer there is provided an adhesive layer 14 for securing the second sheet 16 to the base sheet 10. The adhesive layer 14 can contain a dye or ink if desired.

In another embodiment of the invention shown in 65 FIGURE 2 a third layer of transparent plastic sheet 18 is laminated to the previously formed sandwich comprising sheets 10 and 16. As illustrated this is laminated to layer 10 by means of adhesive layer 20 which can, if desired, contain suitable inks, dyes and the like. To produce patterns, layer 10 or 18 can be printed with stripes 70 or the like prior to forming the final lamination.

In the past, considerable commercial success has been

attained for textile threads made in accordance with the techniques described in Prindle and Lacy Patent 2,714,569. Such products have received wide use in automobile fabric and other textile applications, but their utility in the field of certain other textile applications has been limited by the fact that the aluminum coating utilized in such products is attacked by alkaline dyeing solution so as to partially destroy the laminate and also affect the optical properties of the thread.

The tin coated threads, prepared in accordance with the present invention, overcome this disadvantage of aluminum coated products. The tin coated products are highly resistant to alkaline and other dyeing solutions. Accordingly, the present invention provides an improved laminated thread having excellent resistance to alkaline dyes while still retaining brightness and specular reflectance.

The invention will now be described by way of non-limiting examples thereof.

*Example 1*

In this example of the invention, tin-coated polyethylene terephthalate was prepared by heating a crucible containing tin to a temperature on the order of 1500° C. (as measured by an optical pyrometer with correction for transmission loss through the window of the vacuum coating chamber). The pressure in the vacuum coating chamber was about 60 microns Hg abs. The substrate to be coated (polyethylene terephthalate) was moved over the source of tin vapors at a speed of up to about 1000 feet per minute. The source was an elongated boat extending across the substrate and confining a long molten pool of tin having a dimension of about  $\frac{3}{4}$  of an inch in the direction of motion of the substrate. This gave a calculated coating thickness of approximately 2 millionths of an inch which had a measured resistivity of about 2 to 3 ohms per square. The tin coating was bright and shiny, had a highly specular metallic appearance and adhered strongly to the polyethylene terephthalate sheet. The tin coated sheet was treated in warm moist air for about 4 minutes to oxidize the surface of the tin coating. This sheet was then laminated to another similar sheet and slit to a thread which could be immersed in an alkaline dye bath with no deleterious effect.

*Example 2*

In this example of the invention a sheet of polyvinyl fluoride was coated with tin. In this form of the invention a  $\frac{1}{2}$  mil thick polyvinyl fluoride sheet was cleaned by rinsing with isopropyl alcohol, and then subjecting it to an A.C. glow discharge of 10,000 volts for 10 minutes in a vacuum chamber at a pressure of about 200 microns. A crucible containing tin was then heated to a temperature of about 1500 to 1600° C. (as measured by an optical pyrometer with correction for transmission loss through the window of the vacuum coating chamber). The pressure in the vacuum coating chamber was reduced to about .1 micron Hg abs. The polyvinyl fluoride sheet was exposed to the tin vapors for about  $\frac{1}{2}$  a second and then removed. This gave a coating of about 1 to 2 millionths of an inch thick which had a measured resistivity of about 2 to 5 ohms per square. The tin coating was bright and shiny, had a highly specular metallic appearance and was strongly adherent to the polyvinyl fluoride sheet and could not be removed by the "Scotch" tape test. In this test, pressure-sensitive "Scotch" cellophane tape was pressed on the metallized surface and then rapidly removed.

*Example 3*

In this example tin coated polyethylene terephthalate was prepared by heating the crucible containing tin to a temperature on the order of 1500° C. The pressure in the vacuum coating chamber was maintained in excess of 100 microns and was about 140 microns Hg abs. The substrate was moved over the source of tin vapors at a

speed of about 400 feet per minute. The tin coating produced while being sufficiently thick and adherent was hazy, bluish and did not have a specular metallic appearance.

*Example 4*

In this example the tin coated polyethylene terephthalate was obtained by heating the crucible containing tin to a temperature on the order of 1350° C. The pressure in the vacuum coating chamber was maintained at about 25 microns Hg abs. The substrate was moved over the source of tin vapors at a speed of about 150 feet per minute. The tin coating produced was undesirably thin, brown and nonspecular in appearance.

Numerous types of transparent plastics may be employed in manufacturing the novel thread of the present invention. Examples of such transparent plastic sheets are other polyesters; cellulosic derivatives, such as cellulose acetate and butyrate; polymerized olefins, such as polyethylene and polypropylene; acrylics, vinyl polymers, polyfluoroethylenes obtained from fluorinated ethylenes and copolymers of fluorinated ethylene with unsaturated monomers such as polytetrafluoroethylene and tetrafluoroethylene with chlorotrifluoroethylene.

Since certain changes can be made in the above process and product without departing from the scope of the invention herein involved, it is intended that all matter contained in the above description shall be interpreted as illustrative and not in a limiting sense.

What is claimed is:

1. In the process of producing a vacuum deposited coating of tin on a flexible nonmetallic substrate the improvement which comprises moving said substrate past a source of tin vapors in a vacuum chamber evacuated to a pressure below about 100 microns Hg abs. while heating molten tin in said source to a temperature in excess of 1400° C., condensing said high temperature tin vapors on the substrate to form a dense, shiny adherent tin coating on the substrate, exposing said substrate to the tin vapors for a sufficient time to provide a tin coating of less than about 5 microinches and oxidizing the tin coating by exposing the freshly-deposited tin coating to condensing steam.

2. In the process of producing a vacuum deposited coating of tin on a plastic substrate, the improvement which comprises moving said substrate past a source of tin vapors in a vacuum chamber evacuated to a pressure below about 100 microns Hg abs. while heating molten tin in said source to a temperature in excess of 1400° C., condensing said high temperature tin vapors on the substrate to form a dense, shiny adherent tin coating on the substrate and moving said substrate at a sufficient rate to provide a thickness of the tin coating in excess of about .5 microinch, and oxidizing said tin coating to provide scuff resistance substantially immediately after deposition of said tin coating by exposing the freshly-deposited tin coating to dry steam.

3. In the process of depositing a coating of tin on a flexible substrate in a vacuum chamber, the improvement which comprises evacuating the chamber to a pressure below about 100 microns Hg abs., heating molten tin in a container to a temperature in excess of 1400° C. to provide high temperature tin vapors, condensing said tin vapors on the substrate to form a dense, shiny adherent tin coating, and subjecting said tin coating to heated moist air.

4. In the process of producing a vacuum deposited coating of tin on a flexible nonmetallic substrate, the improvement which comprises moving said substrate past a source of tin vapors in a vacuum chamber evacuated to a pressure below about 100 microns Hg abs. while heating molten tin in said source to a sufficiently high temperature above 1400° C. to provide an evaporation rate of tin in excess of about 2 grams per minute per square inch of molten tin surface, condensing the tin vapors on the substrate to form a dense, shiny adherent tin coating on

the substrate and moving said substrate at a sufficient rate to provide a thickness of the tin coating of between 1 and 5 microinches, and oxidizing said tin coating to provide scuff resistance substantially immediately after deposition of said tin coating by exposing the freshly-deposited tin coating to hot humid air.

5. In the process of producing a vacuum deposited coating of tin on a flexible paper substrate the improvement which comprises moving said substrate past a source of tin vapors in a vacuum chamber evacuated to a pressure below about 100 microns Hg abs. while heating molten tin in said source to a temperature in excess of 1400° C., condensing said high temperature tin vapors on the substrate to form a dense, shiny adherent tin coating on the substrate and moving said substrate at a sufficient rate to provide a thickness of the tin coating of between 1 and 5 microinches, and exposing the freshly-deposited tin coating to condensing steam.

References Cited by the Examiner

UNITED STATES PATENTS

2,039,372 5/1936 Wickmann ----- 117—107  
2,482,054 9/1949 Colbert et al. ----- 117—107

|    |           |         |                     |           |
|----|-----------|---------|---------------------|-----------|
| 5  | 2,665,223 | 1/1954  | Clough et al. ----- | 117—107   |
|    | 2,812,270 | 11/1957 | Alexander -----     | 117—107   |
|    | 2,975,075 | 3/1961  | Beese -----         | 117—107   |
|    | 2,996,410 | 8/1961  | Hnilicka -----      | 117—107.1 |
|    | 3,011,919 | 12/1961 | Niklas -----        | 117—107   |
| 10 | 3,013,919 | 12/1961 | Bialy -----         | 154—53.6  |
|    | 3,028,281 | 4/1962  | Karass -----        | 154—53.6  |
|    | 3,036,933 | 5/1962  | Caswell -----       | 117—107   |

OTHER REFERENCES

Kubaschewski et al.: Oxidation of Metals and Alloys (1953), Academic Press, New York (pages 208 to 210 relied on).

Powell et al.: "Vapor Plating," John Wiley and Sons (1955), pp. 36—37 relied on.

RICHARD D. NEVIUS, *Primary Examiner.*

20 JOSEPH B. SPENCER, *Examiner.*

R. E. HOWARD, A. GOLIAN, *Assistant Examiners.*